

1

2,739,128

## FILM-FORMING COMPOSITIONS

Nicholas M. Adams, Chicago, Ill.

No Drawing. Application March 23, 1951,  
Serial No. 217,305

5 Claims. (Cl. 252—49.6)

The invention is concerned with film-forming compositions, and more particularly it relates to the forming of films on metal surfaces, which films have a protective action and are excellently adapted for use in metal configurating operations.

In cold drawing, forming and other cold shaping operations on metal bodies such as sheet, plate, rod and wire, it is important that the operation be so conducted that no scoring or tearing of the metal occurs under the high pressures employed. In conventional practice both the work piece and the tools such as dies or rolls are coated with some film-forming composition or lubricant throughout the configurating operation. Many types of film-forming compositions and lubricants are employed in industry for this purpose. Long experience has shown, however, that a given composition, while excellent with certain operations and metals, often is wholly unsuitable when the work conditions or metal is changed. Although no universally satisfactory composition has been found for general use in cold forming operations, there are certain well-known characteristics which such a composition should have. The utility of the composition of the present invention can be evaluated in part by the extent to which it is shown to possess these characteristics.

For maximum over-all utility the film-forming composition should greatly reduce the friction between the sliding surfaces of the work piece and the tool. This property is dependent not alone on the lubricating properties of the composition under the prevailing conditions, but also upon the film strength as well. The film strength must be sufficient to avoid mechanical breakdown under the high pressures employed, and to maintain the desired properties under the rise in temperature on the surfaces of the sliding metal members during the configurating operation.

Aside from these essential requisites, there are other properties which are desirable in film-forming compositions of this nature. Among these are the ease of its application to, and removal from, the work piece and tool, its spreading power and its adhesiveness to metal surfaces. Also the composition should be stable, and maintain its useful properties without deterioration from chemical change or separation of constituents during storage. The composition should be substantially inert to the metal of the work piece and the tool, to prevent corrosion of these members. Finally, it should be clean to handle and use, so that the serious housekeeping problems associated with a majority of compositions presently in use may be avoided.

The film-forming compositions of the invention, as will be shown by specific examples of their use, satisfy each of the forelisted requisites, and in addition have other unique properties which render them particularly suitable for use in cold forming operations, and for other purposes.

The invention lies primarily in the finding that certain silicones exert a cooperative effect in combination with particular materials of extreme pressure characteristics,

2

to provide film compositions of highly tenacious adherence to surfaces, and of other exceptional qualities. These films can be applied uniformly to metal or other surfaces through the medium of a suitable solvent for the two components, or by means of an emulsion in another carrier material. A solvent of low temperature volatility is preferable, where formation of a fast drying film is desired, but for some purposes a solvent of slower evaporation rate may be more suitable.

10 The polymeric silicones or polyorganosiloxanes are ordinarily prepared in a partially polymerized form by the hydrolysis of organosilanes which contain at least two hydrolyzable substituents on their silicon atoms, such as hydrogen, halogens and alkoxy radicals, the remaining valances of the silicon atoms being satisfied by organic radicals joined to the silicon through carbon atoms. The intermediate products of hydrolysis are organosilanol, with hydroxy groups directly attached to the silicon, and these condense immediately, or very readily, to form the partially polymerized silicones with the characteristic Si—O—Si bond structure.

20 Among a great many polysiloxane derivatives which may be operative for the purpose of this invention, my investigations to date indicate a preferred action in alkyl polysiloxanes as derived from hydrolysis of the corresponding alkyl halogenosilanes or mixtures of these with alkoxy silanes. For example, a composition made by hydrolyzing and condensing a mixture of amyl trichlorosilane and triethoxysilane, in relative proportions respectively of about 5 to 1 parts by weight, has given excellent results for the purpose intended. This polysiloxane was condensed to the point of forming a viscous liquid, of a chemical structure containing certain Si—H— bonds, as well as similarly bonded alkyl groups, the former bonding being derived from the triethoxysilane starter. Another polymer quite suitable in the invention is one made from ethyl dichlorosilane as the sole starter material. This product was completely hydrolyzed, and partially condensed, so that the final composition was essentially a mixture of the groupings  $[(C_2H_5)HSiO]_n$  and



30 The presence of Si—H bonds is also evident in this polysiloxane, and there is some evidence that this internal structure in the polymer molecule may in part account for the effectiveness in the invention of both materials as described.

40 The second important component of the new composition comprises a material, as already indicated, which has been known and used in extreme pressure lubrication, usually as an additive to mineral oils. Among a great many of such compounds now available, halogenated aliphatic materials, such as the chlorinated paraffin waxes and fatty acid derivatives have proven especially useful. Preferably the extreme pressure component should be one which may tend to decompose at the metal temperatures encountered in deep drawing, such temperatures often being in the neighborhood of 250° C. to 300° C. Paraffin waxes chlorinated to an extent of 30% to 40% by weight have been used successfully in many formulations.

50 The solvent or emulsifying ingredient of the completely blended mixture serves essentially as a carrier to enable ready application of a thin, and uniform, layer of the essential film components to the metal surface. Many known solvents may be useful in this capacity, provided they are compatible with the other ingredients, and produce a homogeneous liquid solution. A volatile solvent is desirable for a rapid dry film application, and a compound solvent to greases and oils has advantages, as will be described later. Of many solvents tested my present preference is for compounds like trichloroethylene, petro-

leum ether, or mineral spirits of about 105° F. flash point.

With regard to the relative proportions in the final film-forming composition, this too can be varied considerably, but in general about one part by weight of the polysiloxane to three or four parts or more of the chlorinated aliphatic compound will produce the desired effect, this mixture in turn being incorporated in the solvent in a total weight amount of from about 5% to 10%. A more specific satisfactory formula has consisted of 20 grams of the previously-described copolymer of amyl trichlorosilane and triethoxsilane, 70 grams of a 40% chlorinated paraffin wax, and 1000 cc. (1455 grams) of trichloroethylene. Substitution for the polysiloxane of the product made directly from ethyl dichlorosilane, in the same relative proportion, also has provided a very effective film-forming composition. Additives of various sort, for inhibitory or other purposes, may be incorporated in the formulae described, and in working with wet films, an oil, like hydrogenated castor oil, or fatty acids and their derivatives, may be added in small amounts to improve slippage.

As previously indicated, a most valuable present-known use for the films of the invention is in metal forming operations which now will be described more in detail.

The blended composition, as it will normally be used, may readily be applied to metal members, as by wiping it on the work piece just prior to the forming operation. Due to the fast evaporation of the solvent, the film is formed in a matter of seconds and there is no objectionable delay between application of the composition and the subsequent shaping operation. If desired, and for many operations it may be preferred, the film may be applied long prior to the shaping operation, and because of its high tenacity and adhesiveness it will remain unimpaired for extended periods. The pre-applied film will also serve to protect the surface of the metal and keep it in such condition that the shaping operation may be performed without additional treatment.

In large scale operations, the metal to be shaped may be advantageously coated with the film-forming composition of the invention at the sheet rolling mill, and subsequently used by the cold forming plant as received from the mill, without further treatment. Due to the oil dissolving properties of the solvent component of the composition, the coating of metal sheet at the mill is greatly facilitated. Oil coated sheets as normally prepared at the mill need only be dipped or continuously passed through a bath of the film-forming composition, in which step the oil on the surface of the sheets is dissolved and combined with a coating of the film-forming composition. Upon evaporation of the solvent, an almost instantaneous occurrence, a lasting film forms on the surface of the metal sheet, which film protects the sheet so effectively that even after prolonged storage the sheet is in an entirely satisfactory condition for cold shaping operations without further treatment or lubrication.

The new film composition is economical to use because of its excellent spreading properties. In many tests it has been found that surface areas of 550 square feet and larger may be satisfactorily coated with a single pound of the composition. Due to the extreme thinness of the applied film, subsequent cleaning of the sheet after the shaping operation is unnecessary and often undesirable. This factor improves housekeeping and effects further economies in the use of the composition. However, since the film is a non-conductor of electricity it may be desirable in some operations, as for example electroplating, to remove the film. This may be done by any well-known dissolving process, as, for example, by dissolving the film in a bath of the solvent in the film-forming composition of the invention.

The film has been employed in comparative cold shaping tests with standard procedures in full scale commercial operations. In all of these tests the composition of the

invention has been found to be entirely satisfactory, and equal, or superior, in performance to the materials heretofore employed. In those instances wherein the customary procedure, due to long experience, was satisfactory from the cold shaping aspects of the problem, the composition of the invention was also equally satisfactory, and in addition was easier in its method of application, as well as more desirable and economical, in that no cleaning operation was required subsequent to the cold forming operation.

Under the particularly severe conditions of cold drawing operations an important property of the film-forming material lies in its ability to prevent "firing" of the die. "Firing" of the die occurs when a small flake of metal welds itself to the die. On each successive draw the welded flake scores the work piece and becomes larger, thus necessitating a shutdown to clean the die. Another property of considerable importance in the cold drawing of metals is the degree of "hold back" exhibited by the film-forming compound or lubricant employed. The effect of "hold back" can be readily shown by employing the film on a work piece or blank whereon a flange is obtained in the drawing operation. The greater the degree of "hold back" exhibited by the film the larger the flange will be. Excessive "hold back" will cause the blank to fracture. In practically all but easy drawing operations on light sheet there is a pressure pad associated with the die, which clamps the outer edge of the blank to the die prior to the punch contacting the blank. The purpose of the pad is to prevent wrinkling of the edges of the blank. However, by varying the pressure on the pad the width of the flange formed in the operation may be varied. Accordingly, the "hold back" of the film must be within the range which can be controlled by adjustment of the pressure pad.

The film of the invention was employed in comparative tests on a commercial scale on the cold drawing of stainless steel coffee pots, wherein dry soap was the conventional lubricant. In the first three tests the polysiloxane component of the composition was a copolymer of 80 mol per cent amyl trichlorosilane and 20 mol per cent triethoxsilane. In the fourth tests the polysiloxane employed was an ethyl dichlorosilane polymer. In all four tests the extreme pressure additive was a chlorinated paraffin wax containing about 40% chlorine and the solvent was trichloroethylene. The ratio of the silicone to the extreme pressure component was 1 to 2 in test No. 1; 1 to 5 in test No. 2; 1 to 15 in test No. 3; and 1 to 5 in test No. 4. After evaporation of the solvent the film formed in all tests had excellent anchorage to the metal surface. Upon heating test strips of the metal the film held firm to the metal in tests Nos. 1 and 2 but had a tendency to run off the metal in tests Nos. 3 and 4. The wetting and tenacity of the film was satisfactory in all tests but was exceptionally high in tests Nos. 1 and 2. Under standard operating conditions the drawing characteristics of the film-coated metal in each of the four tests was excellent. In none of the tests was there any galling or seizure and the surface finish on the completed articles was bright and unmarred. The soap used in the prior standard practice is soluble in water and somewhat hygroscopic, whereas the film of the invention is not. For this reason the steel coated with soap had to be drawn soon after its application, but blanks coated with the film of the invention, for periods of up to four months and longer, have been drawn satisfactorily. In addition the soap used in the prior practice had to be washed off subsequent to the drawing operation. This step is entirely eliminated with the metal coated with the film of the invention.

In many cold forming operations it is necessary to anneal the metal blank between successive working stages. With some materials used in the prior art such as oil and soap this intermediate annealing operation results in carbonizing and staining the metal unless a cleaning

operation is associated with each anneal. By employing the composition of the invention intermediate annealing operations neither carbonize nor stain the coated blanks. This advantage greatly facilitates many cold forming operations by effecting economies in both time and labor.

Similar tests on commercial scale deep drawing of toaster parts, oil seal rings, and many other articles confirm the above observations.

As an example of another application of the film-forming composition of the invention in cold working operations, it has been found that sheet coated with the composition of the invention exhibits superior cold rolling characteristics over sheet not so treated. In a specific application 0.097 inch thick hot rolled carbon steel was coated with the composition of the invention and cold rolled to a thickness of 0.010 inch in seven passes through the rolls. Normally ten to twelve passes have been required in standard practice. In addition the film coated sheet had a cleaner and brighter surface than sheet rolled by the standard practice.

The examples herein given of the methods of employing the film-forming composition of the invention are intended as illustrative examples only and not intended in any manner to limit the scope of the invention as defined in the appended claims.

What is claimed is:

1. A composition adapted to form strongly adherent films on metal surfaces comprising a polyorganosiloxane having alkyl substituents and hydrogen bonded to the silicon atoms, a chlorinated paraffin wax of extreme pressure lubrication characteristics, and a readily volatile solvent carrier for the aforesaid components, the first two components being in relative proportions respectively of one part to at least three parts, by weight, with the total amount of both components constituting from 5% to 10%, by weight, of the entire solution.

2. A composition adapted to form strongly adherent films on metal surfaces comprising a polyorganosiloxane which is a copolymer of amyl trichlorosilane and triethoxysilane, a chlorinated paraffin wax containing about 30% to 40% chlorine, and a readily volatile solvent carrier for the aforesaid components, the first two components being in relative proportions respectively of one part to at least three parts, by weight, with the total

30

35

40

45

amount of both components constituting from 5% to 10%, by weight, of the entire solution.

3. A composition adapted to form strongly adherent films on metal surfaces comprising a polyorganosiloxane derived from the condensation of ethyl dichlorosilane, a chlorinated paraffin wax containing about 30% to 40% chlorine, and a readily volatile solvent carrier for the aforesaid components, the first two components being in relative proportions respectively of one part to at least three parts, by weight, with the total amount of both components constituting from 5% to 10%, by weight, of the entire solution.

4. A composition adapted to form strongly adherent films on metal surfaces comprising a polyorganosiloxane which is a copolymer of amyl trichlorosilane and triethoxysilane, a chlorinated paraffin wax containing about 40% chlorine, and a solvent of trichloroethylene, the first two components being in relative proportions respectively of one part to at least three parts by weight, with the total amount of both components constituting from 5% to 10% by weight of the complete solution.

5. A composition adapted to form strongly adherent films on metal surfaces comprising one part of a polyorganosiloxane derived from the condensation of ethyl dichlorosilane, to at least three parts of a chlorinated paraffin wax containing about 40% chlorine, and a solvent of trichloroethylene in amounts to produce a 5% to 10% total weight solution of the first two components.

#### References Cited in the file of this patent

##### UNITED STATES PATENTS

|           |                |                |
|-----------|----------------|----------------|
| 1,991,395 | Kocour         | Feb. 19, 1935  |
| 2,126,590 | Valentine      | Aug. 9, 1938   |
| 2,223,037 | Ihrig          | Nov. 26, 1940  |
| 2,329,731 | Spring         | Sept. 21, 1943 |
| 2,406,971 | Sowa           | Sept. 3, 1946  |
| 2,470,062 | Whitbeck       | May 10, 1949   |
| 2,471,850 | Wilcock        | May 31, 1949   |
| 2,613,626 | Whitney        | Oct. 14, 1952  |
| 2,623,019 | Wilcock et al. | Dec. 23, 1952  |

##### OTHER REFERENCES

The Modern Industrial Press, pages 6, 8, 20, September 1947.